

July 9, 1929.

A. C. BUNKER

1,719,829

## METHOD FOR PRODUCING SQUIRREL CAGE ROTORS

Filed Jan. 5, 1927

Fig. 1



Fig. 2



Fig. 3



INVENTOR  
*Arthur C. Bunker*  
BY  
*Cooper, Kerr & Dunham*  
HIS ATTORNEYS

## UNITED STATES PATENT OFFICE.

ARTHUR C. BUNKER, OF MONTCLAIR, NEW JERSEY, ASSIGNOR TO CROCKER-WHEELER ELECTRIC MANUFACTURING COMPANY, OF AMPERE, NEW JERSEY, A CORPORATION OF NEW JERSEY.

## METHOD FOR PRODUCING SQUIRREL-CAGE ROTORS.

Application filed January 5, 1927. Serial No. 159,042.

This invention relates to induction motors and more particularly to squirrel-cage rotors and to a method of producing the same.

In the manufacture of rotors of the squirrel-cage type it is desirable to obtain a complete and perfect union of the ends of the conducting bars with the short-circuiting rings or collars for the two-fold purpose of obtaining highest conducting efficiency and maximum strength at the points of connection. It is among the purposes of my invention to provide a method by which a rotor may be obtained which is characterized by accomplishment of this two-fold purpose and which is productive of an article embodying the most perfect construction of a squirrel-cage conducting frame.

Other objects and advantages will be pointed out hereinafter in the specification and in the drawings, in which:

Fig. 1 is a pictorial section of a rotor taken along its axis of rotation, the upper short-circuiting ring being finished and the lower short-circuiting ring being molten and in the process of being welded to the ends of conducting bars.

Fig. 2 is an end view of a rotor with half of a short-circuiting ring cut away.

Fig. 3 diagrammatically illustrates a polished section on line 3—3 of Fig. 2.

My method involves obtaining a perfect weld between each end of a conducting bar 10 and the short-circuiting ring 11 with which it is connected. To accomplish this operation, a mould, 12, for a short-circuiting ring 11 is provided for the purpose of receiving the molten metal and giving it its finished form. The ends of the conducting bars 10 are finished into a plurality of points, 13, 14, in order that the molten metal will be pierced in several places thereby insuring a large contacting surface for the molten metal to affect as well as render it possible for a length 15 of the uncut end of the bar 16 to come into contact with the hot clear metal 17. I have illustrated the plurality of points at one end of a conducting bar in the number of two, which may be of the same or of different lengths, and each end of a single conducting bar is finished in a like manner.

The re-entrant opening 17 cut out at the base of the points has a neck which is relatively smaller across its throat than the width of the area immediately within its

throat. The edges and walls of the points 13, 14 are of such smoothness that gas bubbles are not likely to adhere thereto and thus interfere with the welding action or in some other manner cause a poor weld. The re-entrant opening 17 cut out at the base of the points is of sufficient size to permit any gas bubbles that should gather there to not impair the efficiency of the weld of the uncut immersed portions of the end of the conducting bar with the ring.

Another and important purpose of the reentrant opening 17 is to provide a positive locking relation between the conducting rod 10 and the short-circuiting ring 11 whereby, should there be any weakness or failure in the weld of any one conducting rod, nevertheless there would exist a positive and rigid connection between the conducting rod and the ring where the particular defective or incomplete welding exists. Such precaution is desirable because such a condition as the cooling or solidification of one section of a ring at a different time than another section of the ring may occur to the detriment of obtaining a perfect weld of one or more of the ends of the conducting bars with a ring.

In effect, the positive connection comprises an anchor lug 18 extending from and forming a part of the body portion of short-circuiting ring 11 and engaging with a conducting bar 10 through the co-relation of the walls of the re-entrant opening 17. As has been stated hereinbefore, the re-entrant opening 17 is of sufficient size to permit gas bubbles to gather therein, and whatever bubbles might gather would remain close to the looped inner surface of the confined area and in no way interfere with the formation or effectiveness of the anchor lug 18. Features of my invention which concern structural improvements are described and claimed in a divisional application bearing the Serial Number 315,116.

The method of making the squirrel cage rotor comprises selecting the desired number of conducting rods 10 and finishing them into lengths having ends of the general character and form already set forth. These bars must then be mounted in such a manner as to support them in the relative positions (Fig. 2) that they are to maintain ultimately. This may be accomplished in any way desired, but in small units it is con-

venient to fit each bar within its groove or recess 19 in the core 20. In fitting each bar within a recess 19 a suitable tool may be brought to bear upon the rounded wall portion at the base of the re-entrant opening 17 whereby forces may be applied to the bar without causing damage to points 13, 14. The core, as is well understood, may be made up of laminæ and the whole unit 10 may be conveniently handled by the rotor shaft 21 to which the core is fitted. In the event that the core 20 is not utilized for supporting the conducting bars, the conducting bars would be adjusted and fitted to the 15 core after one of the short circuiting rings has been cast and welded to the conducting bars.

With the conducting bars supported by suitable means, or by the core, the whole assembly 20 is lowered in a vertical direction until the ends of the conducting rods are immersed within the molten metal 16 within the mould 12 substantially as illustrated in Fig. 1. The mould is of such dimensions 25 as to form a short circuiting ring 11. The two points 13, 14 of each rod will pierce the surface of the molten metal and will permit the entry of a bar 10 within the body of the molten metal without producing a 30 substantial derangement in the general pointed outline of the end of a bar.

Fig. 3 is intended to illustrate, diagrammatically, the welded relation of a rod with a ring. This illustration shows a polished 35 section taken on line 3—3 of Fig. 2. The rod and the section of ring is of one piece and the dotted outline of the end of the rod discerns a border line of the two pieces. The heat given off by the molten metal has fused 40 the portion of the end of the rod with which the molten metal has come into contact with the result that the general outline of the end of the rod is maintained, though in an altered form and the two members are one and in- 45 separable.

For concluding the manufacture of the squirrel-cage rotor, the core is positioned in place, if that step has not been completed already, and all of the ends on the other 50 side of the core are immersed within a ring of molten metal in the manner described hereinbefore. This step of the method is pictorially illustrated in Fig. 1. The care incident to the proper carrying out of this 55 step of the process is the same as has been described in the casting and welding of the first ring to the other ends of the conducting rods.

I am aware that the principles of my 60 method may be utilized in many ways, for example, without assembling or making the core until the conducting frame comprising the conducting bars and short-circuiting rings is completed, and that the ends of the 65 conducting bars may be finished in a modi-

fied form other than that specifically illustrated or described.

For these and other reasons I do not restrict myself in the foregoing or other particulars, but contemplate such alterations 70 and modifications within the scope of the appended claims as may be found advisable.

I claim:

1. The method of making a squirrel-cage rotor comprising, finishing each end of a 75 plurality of conducting bars into a plurality of points, supporting each bar in its ultimate position relative to each other, immersing the points of one set of ends into a ring of molten metal, and welding the ends 80 of the rods with the ring formed by the molten metal by the heat of the molten metal.

2. The method of making a squirrel-cage rotor comprising, finishing each end of a 85 plurality of conducting bars into a plurality of points and a reentrant opening, positioning each bar within a core, immersing all of the ends at one side of the core within a ring of molten metal, connecting 90 the ends of the rods with the ring by cooling action, immersing all of the ends on the other side of the core within a ring of molten metal, and connecting the latter ends 95 of the rods with the latter ring by cooling action.

3. The method of welding together two pieces of similar metallic material comprising, finishing into a plurality of points, the portion of one of the two pieces which is to 100 be welded with the second piece, reducing the material to comprise the second piece into a molten state, immersing into the molten material the portion of the first mentioned piece which is to be welded with the second piece, and permitting the molten material of the second piece to solidify with the said portion of the first mentioned piece 105 immersed therein.

4. The method of welding together two 110 pieces of metal comprising, finishing the end of one of the pieces of metal with a plurality of pointed extremities, forming intermediate each pointed extremity a reentrant opening having a relatively small throat, 115 reducing the other piece of metal to a molten state, immersing the pointed extremity of the first named piece of metal into the molten metal to such a depth that the molten metal will flow into the reentrant opening, 120 and permitting the molten metal to solidify.

5. The method of making a squirrel-cage winding comprising, finishing each of the ends of a plurality of conducting bars into a plurality of points, mounting said conducting bars in fixed relation to one another, forming a molten metal bath in a mould so shaped as to receive one set of ends of the conducting bars, causing the points of said 125 one set of ends to enter into the molten metal 130

by relative movement of the conducting bars and molten metal bath, and permitting the molten metal bath to solidify.

6. The method of making a squirrel-cage winding on the rotor core of an induction motor which consists in finishing each of the ends of a plurality of conducting bars into a plurality of extremities, disposing the conducting bars in slots circumferentially disposed about the rotor core, immersing the extremities of the conducting bars disposed at one side of the rotor core into a ring-

shaped bath of molten metal as the result of relative movement of the rotor core and bath of molten metal, permitting the molten metal to solidify, immersing the extremities of the conducting bars on the other side of the rotor core into another bath of molten metal, and permitting the latter bath of molten metal to solidify. 15

In testimony whereof I hereto affix my signature.

ARTHUR C. BUNKER.